

June 18, 1935.

F. R. FROST

2,005,338

MAKING COMPOSITE INGOTS

Filed Dec. 14, 1931

2 Sheets-Sheet 1

*Fig. 1.*



*Fig. 2.*



*Fig. 3.*



INVENTOR

Frank R. Frost  
by his attorney

Dykes, Stubbins, Palmer & Blodke

June 18, 1935.

F. R. FROST

2,005,338

MAKING COMPOSITE INGOTS

Filed Dec. 14, 1931

2 Sheets-Sheet 2

*Fig. 4.*



*Fig. 5.*



*Fig. 6.*



*Fig. 7.*



*Fig. 8.*



*Fig. 9.*



INVENTOR

Frank R. Frost

by his attorneys

Bynes, Stabbins, Parmenter & Blumho

## UNITED STATES PATENT OFFICE

2,005,338

## MAKING COMPOSITE INGOTS

Frank R. Frost, Pittsburgh, Pa., assignor to  
Superior Steel Corporation, Pittsburgh, Pa., a  
corporation of Virginia

Application December 14, 1931, Serial No. 580,747

2 Claims. (Cl. 22—203)

The present invention relates to the making of composite ingots, and more especially to the making of bimetallic ingots. One of the elements of the ingot is formed or placed in the mold and a molten metal forming the other element of the ingot is cast against the first element by centrifugal force. This is preferably accomplished by a centrifugal casting table which forms an annular ingot or a series of ingot units arranged in an annulus, whereby relatively long ingots are secured having the dissimilar metal elements lying longitudinally of the ingot, so as to form convenient ingots for rolling into strip or sheet.

The advantages of my procedure in casting such ingots will be later more particularly pointed out in connection with the description of the apparatus.

In the drawings, which illustrate the preferred apparatus for carrying out my process,—

Figure 1 is a plan view of a casting table having the portion of the top mold plate broken away;

Figure 2 is a vertical section along the line II—II of Figure 1;

Figure 3 is a perspective view of an annular ingot as removed from the mold;

Figure 4 is a detail transverse vertical section through the ingot and ingot mold illustrating how the facing plate is formed on the ingot; and

Figures 5, 6, 7, 8 and 9 are detail views similar to Figure 4 showing modifications in the formation of the ingot.

In the illustrated embodiment of the apparatus, reference numeral 2 indicates a rotatable casting table. This table consists of a flat base plate 3 mounted to be driven by a vertical drive shaft 4, and provided with suitable supporting bearings 5. The table 2 is rapidly rotated by any suitable means, illustrated, for example, as an electric motor 6 having suitable driving connections to the shaft 4.

Upstanding from the edge of the table is a rim 7 suitably secured thereto, as by bolts 8. Secured to the top of the rim 7 and projecting inwardly therefrom is the top plate 9 removably fastened to the rim 7 by suitable means such as the bolts 10. The table 3, the annular rim 7, and the removable top plate 9 form an annular mold cavity which is open inwardly along the side face. The table is arranged to be rotated in the direction indicated by the arrow in Figure 1. Molten metal is supplied to the casting table by any suitable means such as the spout 11

which discharges onto the flat face of the table within the annular ingot mold.

In making a bimetallic ingot, as shown, for example, in Figures 2, 3 and 4, a strip 12 of metal which is to form one of the elements of the bimetallic ingot is laid as a liner against the inwardly facing inner face 13 of the ingot mold. This strip is preferably of a length to extend around the circumference of the ingot mold with its two ends in butting contact. The strip 12 is preferably of somewhat less width than the height of the ingot mold, so as to leave a small clearance space above and beneath the edges of the strip, and for this purpose the strip is spaced slightly above the bottom of the ingot mold by means of small metal blocks 14. After the strip 12 is thus positioned in the ingot mold the centrifugal table 2 is rapidly rotated and molten metal run onto the table through the spout 11. The molten metal is thrown centrifugally into the ingot mold and against the strip 12, solidifying to form the other element or body 15 of the ingot. The molten metal, which is forcibly urged outwardly by centrifugal force, flows around the edges of the strip 12 forming locking tongues 16 and 17 cast tightly against the edges of the strip. After the metal is solidified the table is stopped, the top plate 9 taken off, and the ingot 18, which is shown in Figure 3, is removed from the table. If necessary, the outer ring or rim 7 can be taken off in removing the ingot. The ingot 18 is then cut into lengths, as indicated by the division lines 19, to form units or billets 20 which are afterward rolled down to form bimetallic strips or sheets.

The casting apparatus is constructed of suitable size. For example, in making ingots for rolling into strips or sheets, a table about ten feet in diameter is suitable, and an ingot about six inches square is a convenient size for use in rolling mill equipment. In making bimetallic strips or sheets the element formed by the strip or plate 12 is usually thinner than that formed by the cast metal 15, the thinner metal being the more expensive facing material which it is desired to apply to a cheaper backing material. For example, in making bimetallic strip or sheets where corrosion resistant properties are desired, a rolled strip 12 of stainless steel or rustless iron of, say, about one inch thick, is placed in the ingot mold and a layer 15 of about five inches thick ordinary plain carbon steel is cast against the strip 12. When the ingot is rolled down the material of the strip 12 forms a thin corrosion-resistant facing applied to the

- backing of plain carbon steel. The facing material 12 may be a metal known as "stainless steel" or "rustless iron" containing usually about 12 to 18 per cent chromium with the balance iron and 5 low carbon content, or a facing material of alloy of about 18 per cent chromium, 8 per cent nickel, with the balance iron and low carbon, may be employed. The backing material 15 is preferably of plain carbon steel which is used because 10 of its cheapness and physical properties. A mild open hearth steel may be employed for making sheets for drawing purposes, or a higher carbon spring steel may be employed in making stock for purposes such as that of automobile 15 bumpers. While the two elements of the composite ingot have been specifically described as of plain carbon steel and stainless steel or rustless iron, other metals may be used in forming the composite or bimetallic ingot.
- 20 The centrifugal process of casting, as herein applied is peculiarly adapted for making bimetallic ingots from which billets may be cut for rolling purposes. The welding of the facing metal to the backing metal, and particularly 25 where a preformed strip of facing metal is laid in the ingot mold, is primarily accomplished during the rolling of the billets into strip or sheet form. For this purpose the billets are heated in a reheating furnace to a suitable rolling temperature and are then put through the rolling mill rolls which reduce the billets into strip or sheet form and at the same time, by means of the rolling pressure, weld the facing layer to the 30 backing layer so as to form an integral bimetallic body. In order to accomplish proper rolling and welding, the strip of facing material 12 should be firmly held to the backing material 15 and the edges of the strip should be sealed to the 35 backing material so as to exclude the atmosphere or furnace gases which, if they should penetrate between the adjacent faces of the strip 12 and backing 15, would oxidize the material and interfere with good welding. The tongues 40 16 and 17 accomplish this purpose. When the molten metal is poured onto the centrifugal table it is projected violently outwardly against the facing strip 12 and is caused to flow under the strong centrifugal force around the edges of the strip to form the locking tongues 16 and 17. 45 Ordinarily the edges of the strip are sufficiently irregular so that a tight lock is formed between the tongues 16 and 17 and the edges of the strip so as to hold it securely for the rolling operation. The tongues also form a seal to exclude the 50 atmosphere from the juncture between the inner faces of the strip 12 and the cast metal backing 15.
- 55 The strong pressure of the metal 15 as it is cast against the strip 12 also tends to expel any air from being entrapped between the strip 12 and the body of backing metal 15, and to force the backing metal 15 into intimate surface contact with the strip 12. Since the metal 15 is cast under strong centrifugal force, any gases 60 are squeezed from the molten metal inwardly, and the metal of the body portion 15, particularly the outer portions of such metal which are next to the strip 12, are effectively freed from gases and compacted into a dense condition.
- 65 70 The compacted gas-free metal which is forced strongly against the strip 12 gives optimum conditions for the welding of the metal 15 to the strip 12. It will be readily seen that it is of material advantage to have the densest gas-free portion of the metal body 15 against the

facing layer 12 which is to be united to the backing layer by the welding operation.

The bimetallic ingots or billets produced by this casting operation are particularly well adapted for rolling into sheets or strips. Any variation in the density or like characteristics of the cast body of backing metal 15 will occur along a direction normal to the facing plate 12, or in the direction of the height of the billet as it is rolled in the rolling mill. The sheets 10 or strips rolled from such billets will therefore tend to be uniform throughout their length and breadth. Considering, because of the acceleration of gravity in that direction, the face 13 of the ingot mold to be the effective "bottom" 15 of the mold, the ingot, in effect, has a "bottom" of relatively large area formed of the plate 12 against which the dense "bottom" metal of the body portion 15 of the ingot is uniformly distributed. The other face of the body portion 20 or what might be considered to be the "top" portion of the ingot where the metal may be less dense or where segregation is most likely to occur, is farthest removed from the welding contact with the facing plate 12, and in a place 25 where such metal can be readily removed if desired.

In the making of bimetallic articles having a chrome iron facing and a plain carbon steel backing, there is a tendency during the welding 30 operation for the carbon from the plain carbon steel to migrate into the chrome iron facing and reduce its corrosion-resisting properties. The chromium has greater affinity for carbon than the iron. In making bimetallic articles, particularly those in which a low carbon chrome iron facing is desired upon a high carbon steel backing, such as required for automobile bumpers, there is a strong tendency during the heating and rolling operations for carbon to migrate 35 from the steel backing into the chromium iron facing. This may be prevented by placing over the inner face of the chrome iron strip 12 a thin sheet 21 of an exceptionally low carbon iron, such, for example, as ingot iron or wrought 40 iron, as illustrated in Figure 5, which will form a barrier to prevent absorption of carbon by the chrome iron facing from the carbon steel backing. The strip 21 may be about one-eighth 45 inch thick and is preferably positioned on the 50 facing material 12 by spot welding. The use of such barrier sheet of exceptionally low carbon material for the prevention of carbon migration is described and claimed in my application Serial No. 580,748, filed of even date herewith. 55

In Figure 6 the liner or strip of facing material 12<sup>a</sup> is shown as having beveled edges around which the metal of the cast body 15 flows to form dovetail locking tongues 16<sup>a</sup> and 17<sup>a</sup> in order to give a more secure lock between the 60 facing plate 12<sup>a</sup> and the body of backing metal 15<sup>a</sup>.

In Figure 7 the same beveled liner or facing strip 12 is shown but with a thin sheet 21<sup>a</sup> of exceptionally low carbon iron, such as ingot iron 65 or wrought iron, interposed between the facing material 12<sup>a</sup> which is preferably a low carbon chrome iron and the backing material 15<sup>a</sup> which is preferably plain carbon steel.

While the liner 12 which lies against the face 70 13 of the ingot mold, as shown in Figures 4, 5, 6 and 7, is formed of a strip of metal laid into the ingot mold, the liner may be otherwise formed. In Figure 8 I have illustrated the liner 75 12<sup>b</sup> as formed by casting the facing metal first

in the ingot mold by the centrifugal casting operation. For example, a small ladle of chrome iron can be first poured through the spout 11 on the rotating centrifugal table and the liner 12<sup>b</sup> cast in place. This can be followed by pouring in a larger ladle of plain carbon steel to form the body 15<sup>b</sup> which is cast against the liner 12<sup>b</sup>. In this case the plain carbon steel may be poured while the chrome steel is still 10 hot and plastic so that at least incipient welding may take place between the two metals, or the chrome steel liner may be allowed to chill before plain carbon steel is cast against it.

In Figure 9 is shown another modification of the process in which the plain carbon steel body 15<sup>c</sup> of the ingot is first centrifugally cast to form a thick liner in the mold and then the facing metal, such as the chrome steel, is cast 15 to form the thin facing layer 12<sup>c</sup> against such liner. As in the modification last described, the second-poured metal may be introduced while the first-poured metal is still somewhat plastic in order to get some welding effect between them, or the first-poured metal may be allowed to completely solidify or to cool somewhat before the second-poured metal is introduced.

While I have specifically described my process with reference to making composite ingots having a rustless iron facing and a plain carbon steel backing, it may be employed in making composite ingots of other metals. It also may be employed in making composite ingots having three or more metal layers if desired.

The composite ingot produced according to the present invention is the subject matter of a divisional application, Serial No. 732,655, filed June 27, 1934.

While the preferred embodiment of the invention has been specifically illustrated and described, it should be understood that the invention is not so limited but may be otherwise embodied and practiced within the scope of the following claims.

I claim:

1. The process of making composite metal ingots, which comprises placing a liner of one metal in an ingot mold, leaving spaces between the edges of the liner and the mold walls, revolving the mold, and introducing another metal in a molten state into the mold so as to cast the molten metal by centrifugal force against the liner and cause the molten metal to enter the spaces around the edges of the liner, so as 20 to form a composite ingot having the liner securely held to the body of metal cast against it.

2. The process of making composite metal ingots which comprises forming a liner against the inwardly facing inner face of the mold and leaving spaces between the edges of the liner and the mold walls, revolving the mold, and introducing molten metal into the revolving mold so as to cast it by centrifugal force against the liner and form a composite ingot having the liner held 25 to the body of the cast metal by tongues of the cast metal formed in the spaces between the edges of the liner and the walls of the mold.

FRANK R. FROST.